

April 16, 1929.

J. H. CHRISTENSEN

1,709,563

COLORED PICTURE AND METHOD OF PRODUCING THE SAME

Filed Jan. 24, 1927

*Fig. 1.*



*Fig. 2.*



*Fig. 3.*



*Fig. 4.*



Jens H. Christensen  
Inventor,  
by Victor W. Dorst  
Attorney

Patented Apr. 16, 1929.

1,709,563

# UNITED STATES PATENT OFFICE.

JENS HERMAN CHRISTENSEN, OF HOLTE, DENMARK.

## COLORED PICTURE AND METHOD OF PRODUCING THE SAME.

Application filed January 24, 1927, Serial No. 163,017, and in Denmark, January 25, 1926.

It is well known that colored pictures can be produced by means of a multicolor screen consisting of small colored elements, but such pictures present good colors in transmitted light only, and photographic plates of this kind are found in the trade. It has also been attempted to use the same principle in pictures which are to be seen in reflected light, it having been attempted to 5 place a colored diapositive made in the manner outlined above upon a reflecting under-layer, but the attained results have been poor, and it is the general belief that the method is appropriate for producing of 10 pictures only which are to be seen in transmitted light.

I have found, however, that it is possible according to the known principle to produce good pictures which can be seen in reflected light, and the conditions which are to be fulfilled, according to practical experiments, when a favorable result shall be attained, are best understood by contemplating the annexed diagrammatical drawing. Figure 1 shows a section through a colored screen picture placed on a white reflecting layer of the commonly used kind and serves only for explaining the invention. Figure 2 represents a section through 20 a similar arrangement, the white layer having a better reflecting property according to the invention. Figures 3 and 4 show further modifications.

*a* designates a section through a carrier of 35 glass or celluloid for the colored elements forming the layer *b*. The elements can for instance be red, green, and blue transparent particles which are mixed with each other. The layer *c* is a panchromatic photographic 40 film, which can be found directly on the layer *b* or if necessary be separated from the same through a thin varnish film *k*, if it is necessary to protect the colored elements against the action of the aqueous baths with 45 which the photographic film must be treated.

The picture is produced by the emulsion film *c* becoming opaque, owing to the silver reduced by the developer opposite the particles the colors of which do not correspond 50 to that which the picture shall present on the place in question. If it be assumed for instance that a purely green object is photographed, the silver will after exposure and known treatment of the plate cover all of the 55 red and the blue elements as indicated on the drawing while the film remains clear

opposite to the green elements *g*, and if the picture is seen in transmitted light an exceedingly brilliant and transparent green color can be obtained.

If now a piece of white paper be laid in contact with the film *c* it was to be expected that this brilliant green picture could be seen in reflected light but in practice a very dark and unpure green picture only is seen.

If the white paper referred to above be provided with a cover of barium sulphate (the commercial baryta paper) or of calcium carbonate, white paint or another commonly used white reflecting substance, the result becomes somewhat better but is far from satisfactory. The matter is namely, that if the green light can enter through an appreciable distance into the reflecting layer, before it is reflected or returned, it is to a 75 considerable extent lost to the picture, it being in such case reflected partly to the sides and a smaller part of the same only through the green color element, through which the light has entered. It is easily 80 understood from Figure 1 of the drawing, that a light ray passing through the layer *d* until the point *f* will to a considerable extent not be reflected through the opening through which it entered, but the light will 85 become lost through absorption in the red and blue neighbouring elements or the silver layer covering the same. If however, the ray is reflected already at the point *h*, in Figure 2, it is seen that practically all of 90 the light will be reflected through the admission aperture and thus be able to act on the eye. It is furthermore seen that the distance within which the light must be reflected for mainly passing through the admission aperture is depending upon the diameter of the latter or of the colored element, and this distance should preferably be less than the diameter of the said aperture. As 95 the colored elements must be so small that they do not disturb the distinctness of the picture, it is very small distances which are in question here, and at the common white reflecting substances the reflection takes place mainly from a greater depth.

In order to produce a white layer which reflects the light as near the surface as necessary I have tried to use strongly light refracting substances such as titan white, lead tungstate etc. mixed with an exceedingly 100 small amount of a binder, and rather favorable results were attained. If the binder was 110

totally omitted the said substances being applied by means of a brush or through dusting in with the same the result was far better, the binder being then replaced by air.

5 Such a layer is, however, of no value in practice having no coherence and being apt to fall off.

It is known that such substances as nitro-cellulose and acetyl cellulose after dissolution in appropriate solvents and after being poured out on a surface upon drying can yield a snow white cover, and such white layer has proved to give a rather favorable effect, but such layers have also often a so 15 small mechanical strength that they are useless in practice. I obtain a better result by adding to 100 cc. 4%—containing collodion 100 cc. toluene and 40 to 80 grams of a white pigment (lead white, titan white or the like).

20 After drying a snow white film is obtained which has a certain mechanical resistance power and is penetrated by numerous air fissures *e* as shown in Figure 4 which augment the reflecting power. If these fissures 25 are filled out for instance through soaking of the film in amyl acetate and drying of the same, the film apparently conserves its whiteness but the reflexion is effected in a much less degree from the surface itself, and when 30 laid against a colored picture of the above mentioned kind a far less brilliant picture is obtained.

In lieu of the above named mixture of colloidion and toluene other solutions of cellulose derivates can be used which are apt to be separated out in a white layer and form air filled fissures on drying.

It has shown to be of little importance whether the reflecting layer be applied directly to the film *c*, for instance through pouring out upon the same and drying, or whether it is found between the layers *a* and *b*, as shown in Figure 3, thus under the layer of colored elements. In the last named case 45 it can be present before the exposure and development.

The said white layer can also be made by pouring out on paper and drying, and it can be pasted on the picture after same is made 50 ready. Care must be taken that the binder used does not fill up the air fissures in the layer. As a binder a weak rubber solution can advantageously be used. Figure 4 shows an arrangement of this kind, the air fissures 55 being designated by *e* and the paper by *p*.

In all of the structures shown in the drawing and herein described, the film which comprises a layer of colored elements *b* covered by a silver containing layer *c*, is brought in 60 contact with the reflecting layer *d* within the

meaning of the claims, whether this be done by placing the layer *d* on a separate backing *p* and then bringing the film in contact therewith as in Figure 4, or by bringing the film in contact with the reflecting layer *d* by 65 pouring same upon the film and drying as previously described.

Having thus fully described my invention I claim as new and desire to secure by Letters Patent:

1. Method of producing colored photographic pictures to be seen in reflected light under use of a film comprising a layer of colored elements covered by a silver containing layer, consisting in bringing the said 75 film in contact with a coherent white layer reflecting the main part of the light within a depth from the surface of the said white layer not exceeding the average diameter of the colored elements. 80

2. Method of producing colored photographic pictures to be seen in reflected light under use of a film comprising a layer of colored elements covered by a silver containing layer, consisting in bringing the said 85 film in contact with a layer of a cellulose derivate which is penetrated by numerous air filled fissures.

3. Method of producing colored photographic pictures to be seen in reflected light 90 under use of a film comprising a layer of colored elements covered by a silver containing layer, consisting in bringing the said film in contact with a layer of a cellulose derivate which is penetrated by numerous air 95 filled fissures and contains a white pigment. 100

4. As an article of manufacture, a colored photographic picture to be seen by reflected light, comprising a layer of colored elements, a silver containing layer and a coherent white layer which reflects the main part of the light within a depth from the surface of the said white layer not exceeding the average diameter of the colored elements. 105

5. As an article of manufacture, a colored photographic picture to be seen by reflected light, comprising a layer of colored elements, a silver containing layer and a layer of a cellulose derivate which is penetrated by numerous air filled fissures. 110

6. As an article of manufacture, a colored photographic picture to be seen by reflected light, comprising a layer of colored elements, a silver containing layer and a layer of a cellulose derivate which is penetrated by numerous air filled fissures and contains a white pigment. 115

In testimony whereof I have affixed my signature.

JENS HERMAN CHRISTENSEN.